

# UNITED STATES PATENT OFFICE.

JAMES F. SALLows, OF KALAMAZOO, MICHIGAN.

## PROCESS OF PRODUCING AND FINISHING GEARS AND OTHER CARBONIZED-STEEL PARTS.

1,282,467.

Specification of Letters Patent. Patented Oct. 22, 1918.

No Drawing.

Application filed December 7, 1917. Serial No. 205,976.

To all whom it may concern:

Be it known that I, JAMES F. SALLows, a citizen of the United States, having residence at Kalamazoo, in the county of Kalamazoo and State of Michigan, have invented certain new and useful Improvements in Processes of Producing and Finishing Gears and other Carbonized-Steel Parts, of which the following is a specification.

10 The purpose of this invention is to provide an improved process for producing hardened steel or carbonized iron parts, such as gears and the like, for avoiding deformation in the process of hardening. It consists in the several steps hereinafter described, as set out in the claim.

Heretofore difficulty has been experienced in producing satisfactory steel or carbonized iron parts requiring accuracy of dimension and form without grinding as the final process of finishing to form and for removing scale, because the usual steps of hardening produce not only internal stresses but also deformation, and tool-finishing cannot be resorted to after the hardening is completed, and the deformations can be corrected only by a process which can be applied to the hardened material; such, for example, as the process of grinding and polishing.

30 I have overcome this difficulty by the following process:

I first produce by forging the article desired in the rough, or of approximately the form and dimension required. I next "rough-machine" the part to a still closer approximation to the form and dimension required. For the third step I case-harden the part, employing the usual means and processes for carbonizing it quite deeply, and upon the conclusion of the carbonizing step, I quench the parts in oil first allowing them to cool in the pots to proper tem-

perature for hardening by the quenching. As the next step, I box the part in carbon 45 dust, that is, inclose it in a box and pack it with carbon dust, and heat the package to proper temperature for annealing, that is to say, about 1400 degrees F., and permit it to remain in the heating furnace a proper length 50 of time to produce the desired refined structure of the casing, and then remove the package from the furnace and allow to cool in the atmosphere, or normally, without unboxing. The next step consists in finish-machining 55 the part to final form.

I then repack in carbon in a box, and reheat to a temperature of 1200 to 1400 degrees F., and remove from the packing and quench the article in oil or water according 60 to the grade of steel required.

The parts produced in this manner are found to have the form and dimensions to which they are finish-machined, without warping or distortion of any sort, and apparently without injurious internal stresses.

I claim:

The process of producing steel or carbonized iron parts comprising the following steps: first, rough-forming the parts; second, rough-machining parts approximately to the form and outline required; third, carbonizing deeply by case hardening process, and quenching in oil; fourth, annealing by boxing in moderately insulating material as 70 carbon dust, heating and allowing to cool normally in the atmosphere without unboxing; fifth, finish-machining; sixth, re-boxing in moderate insulation, re-heating and quenching in oil or water according to the 75 grade of steel required.

In testimony whereof, I have hereunto set my hand at Kalamazoo, Michigan, this 30th day of November, 1917.

JAMES F. SALLows.